

Patented May 11, 1926.

1,584,005

# UNITED STATES PATENT OFFICE.

EMILE BINDSCHEDLER, OF LANSDOWNE, PENNSYLVANIA, AND GEORGE JUER, OF HOPEWELL, VIRGINIA, ASSIGNEES TO TUBIZE ARTIFICIAL SILK COMPANY OF AMERICA, A CORPORATION OF DELAWARE.

## METHOD OF MANUFACTURING ARTIFICIAL SILK AND OTHER PRODUCTS FROM NITROCELLULOSE.

No Drawing.

Application filed July 1, 1924. Serial No. 723,485.

Our invention relates to the known process in which the collodion obtained by dissolving nitrocellulose hydrate in a mixture of ethyl alcohol and ether is given desired form by 5 exuding it through an orifice and the filament or other product thus formed is coagulated by the removal of the solvents.

It has been proposed to coagulate nitrocellulose collodion by passing it into a bath of 10 dilute ethyl alcohol, preferably of a strength varying from 25 to 60%. We have found that to secure clear and lustrous filaments, the coagulating bath should have a strength of at least 40%. We have also discovered 15 that the rate of coagulation in such a bath can be regulated by dissolving in dilute ethyl alcohol a neutral inorganic salt or salts. Such regulation of coagulation can be 20 available of to vary in some degree the character of the product and the operation of the process.

Certain metallic salts, especially haloids, when dissolved in dilute alcohol have in most 25 cases a pronounced retarding effect on the rate of coagulation. We found calcium chloride and magnesium chloride especially well adapted for the purpose, these salts, having a further advantage of being cheap and their aqueous solutions are miscible, 30 to a great extent, with the usual ether-alcohol mixture.

Where acceleration of coagulation is desired, zinc chloride is preferably used because among other reasons, it has the valuable 35 property of being soluble not only in alcohol, but also in ether.

We have availed ourselves of the retarding effect of calcium chloride or similar salt dissolved in dilute alcohol on the coagulation 40 of the exuded filaments to produce a thread of finer denier and we effect this by winding up the filaments at a speed greater than the rate of exudation of the collodion through an orifice, the result being that the still plastic thread is drawn out and made finer before coagulation gives permanent form to it.

By preference we complete the coagulation and extract the salt by passing the thread through a second bath of dilute ethyl alcohol 45 of from 40 to 60° strength, but this is not essential and the thread may be passed directly to the bobin rotating in water which will remove any remaining solvent, alcohol

and salt. The solvents and salt solutions can be easily and almost completely recovered 55 according to well known methods.

We should mention that by varying the temperature of the coagulating bath between 20 and 35° C., a further regulation of the 60 rapidity of coagulation can be effected.

As a specific example of the application by our improved method in such a way as to retard coagulation to produce filaments of fine denier we give the following:

Nitrocellulose hydrate containing from 65 20 to 30% water is dissolved in a mixture of 60 parts ether and 40 parts ethyl alcohol and the collodion so obtained is spun into a coagulation bath consisting of 50% ethyl alcohol in which 20 parts calcium chloride 70 have been dissolved per 100 volume parts. The threads coming out of the orifices in a semi-coagulated state are elongated by tension to the desired fineness and the filaments are washed preferably first with 40% alcohol 75 and finally with water.

After twisting and reeling, the threads are denitrated in the usual manner and clear and lustrous filaments are produced.

The following is a specific example of the 80 application of our invention in case acceleration of the coagulation is desired:

Nitrocellulose hydrate containing 20 to 30% water is dissolved in a mixture of 50 85 parts ether and 50 parts ethyl alcohol and the collodion so formed, is spun into ethyl alcohol of 40% strength in which 50 parts of zinc chloride have been dissolved per 100 volume parts of dilute alcohol, the threads so formed are directly wound on bobbins, rotating in water.

Having now described our invention, what we claim as new and desire to secure by Letters Patent, is:

1. In the process of manufacturing 95 formed products from nitrocellulose hydrate dissolved in alcohol and ether unadmixed with other chemicals by exuding the collodion through an orifice to give form to the product and coagulating the exuded product, 100 the method of regulating coagulation which consists in exuding the collodion into a bath composed of one or more neutral inorganic salts dissolved in dilute alcohol.

2. In the process of manufacturing 105 formed products from nitrocellulose hydrate

dissolved in alcohol and ether by exuding the collodion through an orifice to give form to the product and coagulating the exuded product, the method of regulating coagulation which consists in exuding the collodion into a bath composed of one or more metallic haloids dissolved in dilute alcohol.

3. In the process of manufacturing formed products from nitrocellulose hydrate dissolved in alcohol and ether by exuding the collodion through an orifice to give form to the product and coagulating the exuded product, the method of retarding coagulation which consists in exuding the collodion into a bath composed of calcium chloride dissolved in dilute alcohol.

4. In the method of manufacturing artificial silk from nitrocellulose hydrate dissolved in alcohol and ether unadmixed with other chemicals by exuding the collodion through an orifice and coagulating the filament, the method of retarding the coagulation and producing a filament of fine denier which consists in exuding the collodion filament into a bath of dilute alcohol having dissolved in it neutral inorganic salts which retard coagulation and drawing the filament through said bath at a rate exceeding the

rate of exudation so as to elongate and reduce the denier of the filament. 30

5. In the process of manufacturing formed products from nitrocellulose hydrate dissolved in alcohol and ether unadmixed with other chemicals by exuding the collodion through an orifice to give form to the product and coagulating the exuded product, the method of regulating coagulation which consists in exuding the collodion into a bath composed of one or more neutral inorganic salts dissolved in dilute alcohol of 40 from 40 to 60° strength.

6. In the process of manufacturing formed products from nitrocellulose hydrate dissolved in alcohol and ether unadmixed with other chemicals by exuding the collodion through an orifice to give form to the product and coagulating the exuded product, the method of regulating coagulation which consists in exuding the collodion into a bath composed of one or more neutral inorganic salts dissolved in dilute alcohol and afterwards through a second bath of alcohol diluted to 40 to 60° strength. 45 50

EMILE BINDSCHEDLER.  
GEORGE JUER.